

Patented Dec. 29, 1925.

1,567,277

## UNITED STATES PATENT OFFICE.

ARMAND L. LABBE, OF MURRAY, UTAH, ASSIGNOR TO AMERICAN SMELTING AND REFINING COMPANY, OF NEW YORK, N. Y., A CORPORATION OF NEW JERSEY.

## COMPOSITION FOR ELECTRIC INSULATORS AND METHOD OF PREPARING SAME.

No Drawing.

Application filed August 16, 1921. Serial No. 492,654.

*To all whom it may concern:*

Be it known that I, ARMAND L. LABBE, a citizen of the United States, and resident of Murray, in the county of Salt Lake and 5 State of Utah, have invented certain new and useful Improvements in Composition for Electric Insulators and Methods of Preparing Same, of which the following is a specification.

10 The invention relates in general to an improved insulator for a high tension electric current of the type which may be used to support the weight of some structure thereon and the invention also relates to a new 15 composition of matter for use in forming electric insulators and to a method for forming such insulators.

While the insulator herein disclosed is of 20 general application for use in any situation where it is desired to electrically separate two members having different electrical potentialities, the device illustrated is particularly designed for use in situations where high voltage is used, where the presence of 25 gases containing acid and moisture tend to interfere with the effective operation of insulators of the usual type and where electrodes or other strain inducing parts are apt to crush the supporting insulators if 30 they be made of frail construction.

As one illustration of a situation where the invention is particularly applicable, reference is made to an insulator exposed 35 to the smoke or fumes passing from a metallurgical plant. In such cases it has been usual to mount the bars carrying the conductor on ordinary porcelain insulators. These porcelain insulators have not proven satisfactory and break down after they 40 have been in use for a while. It is believed that this is due to acids and moisture collecting on the surface which form a conductive coating. The current present passes through the coating thus formed, overheats 45 the insulator and breaks the porcelain perhaps due to the unequal heating of the different parts of the same. Insulators made of other materials, such as marble have the objection that they are relatively expensive 50 and also must be wiped off occasionally to remove accumulations but obviously this necessitates the interruption of the functioning of the apparatus in which they are mounted.

55 Accordingly, one of the objects of the

present invention is to provide a simple and inexpensive form of insulator which will possess high dielectric strength and which will maintain its insulating characteristics over a relatively long period of time even under the deleterious conditions incidental to the passing of hot acid gases and moisture past the insulators. 60

Broadly, I attain this object of the invention by molding the insulators of a plastic composition which is formed entirely, or largely, of slack lime and in permitting the formed insulators to harden into any desired form. 65

As slackened lime is frangible and difficult to mold and handle, the invention also contemplates the uniting with the lime, of some body-forming-material together with a suitable binding material for uniting the substances into a body capable of maintaining its configuration even when subjected to disrupting strains. As an illustration of one such body substance reference is made to sand and Portland cement which is excellent as a binder. One composition which 70 has given entire satisfaction comprises slack lime 40%, Portland cement 50% and sand 10% by weight. 75

In preparing the material the lime which should be free of magnesia is slacked for 80 several days so as to insure against cracking of the formed block during the succeeding drying operation. 85

The materials enumerated are forced through a forty mesh screen; mixed into a 90 soft paste and worked by hand into the molds which are preferably made of iron. The composition is allowed to remain in the molds, covered with wet sacks, for several days, about three days being the usual time, at the end of which period they are placed under water for a relatively long time, usually about ten days. At the termination of this water treatment the formed insulators are removed from the molds, dried at 95 atmospheric temperature for about ten days, after which they are subjected to a slow baking operation usually for about ten days and at a temperature of approximately 100 140° F. 105

When making up the insulators, it is found to be an advantage to make them in the form of flat disks comprising a plurality of disks stacked one on the other to form a completed insulator. 110

- The insulator herein disclosed has proven satisfactory in active operation and has an advantage over other similar devices in that it readily takes up both acids and condensed moisture from its environment, without impairing its dielectric efficiency. The lime present reacts with any sulphur-acid gases present to form calcium sulphate which is itself a good dielectric. The insulator disclosed has the further advantage in that it absorbs moisture at relatively low temperatures and liberates the same at the higher temperatures usually present in the gases.
- 15 A still further advantage in the type of insulator herein disclosed is that after it has been punctured by the electric current passing therethrough it can be slowly dried out for a period of about four days and at 20 a temperature of about 160° F. after which treatment its dielectric strength is substantially re-established.

Having thus described my invention, I claim:

1. A process of forming an electrical insulating material for high voltage electric current which consists in mixing slack lime substantially free from magnesia in the proportion of not less than 40% and Portland cement and sand in substantial proportions, said ingredients being mixed together and formed into shape and then baked prior to use for insulating purposes.

2. A composition of matter for use as an electric insulating material comprising slack lime, sand and Portland cement, and in the proportion approximately of lime, forty per cent, sand ten per cent and cement, fifty per cent.

Signed at Murray in the county of Salt Lake and State of Utah this ninth (9th) day of August A. D. 1921.

ARMAND L. LABBE.